# EUROPEAN PATENT SPECIFICATION

(11) **EP 0 151 152 B1**
(45) Date of publication and mention of the grant of the patent: **25.11.1987**
(21) Application number: 84902740.4
(22) Date of filing: 25.06.1984
(51) Int. Cl.: B44C 1/175

(54) **GRAPHICS TRANSFER MEDIUM AND METHOD OF APPLYING GRAPHICS TO A DISPLAY SURFACE**
ÜBERTRAGUNGSMITTEL FÜR GRAPHISCHE DARSTELLUNGEN UND VERFAHREN ZUM ANBRINGEN VON GRAPHISCHEN DARSTELLUNGEN AUF SCHAUFLÄCHEN
SUPPORT DE TRANSFERT GRAPHIQUE ET PROCEDE D'APPLICATION DE MOTIFS GRAPHIQUES SUR UNE SURFACE D'AFFICHAGE

(30) Priority: 01.08.1983 US 519528
(43) Date of publication of application: 14.08.1985
(73) Proprietor: MINNESOTA MINING AND MANUFACTURING COMPANY, St. Paul, Minnesota 55133-3427 (US)
(72) Inventor: STEELMAN, Ronald, S., Saint Paul, MN 55133 (US)
(74) Representative: Baillie, Iain Cameron
(86) International application number: US8400984
(87) International publication number: WO8500560

## Description

### Background Art

Retail businesses often make visual announcements by hand lettering or stenciling display surfaces such as windows or by hanging posters or newspaper advertisements. Such announcements may be unsightly unless an inordinate amount of time is devoted to their creation and application.

Visual announcements may also take the form of decals which may incorporate ornamentation and can be highly attractive. However, decals are expensive to create and difficult to remove. Because water-soak decals tend to be cumbersome, slow to apply, and difficult to position, pressure-sensitive adhesive decals have come into widespread use. However, either the adhesive must he applied in register with the graphics or some mechanism must be provided to separate the adhesive at the precise outline of the graphics. These requirements are particularly difficult to achieve if the graphics have fine detail.

### Disclosure of the Invention

By the method of the invention, graphics having fine detail and quality appearance can be applied with precision to a disllay surficc easily and at remarkably low cost. Simple adjustments in the method permit the transferred graphics to be either difficult or easy to remove from the display surface.

In short, the novel method comprises the sequential streps of
1) applying to a flexible low-adhesion carrier web a coating in the form of graphics, which coating comprises a liquid mixture of
   a) matrix resin,
   b) binder resin, and
   c) light-altering agent,
2) solidifying the coating of graphics,
3) wetting the solidified coating of graphics with a fluid which at least partically dissolves the binder resin and substantially does not attack either the matrix resin or the carrier web,
4) pressing the wet coating of graphics against a display surface,
5) allowing to develop between the coating of graphics and the display surface a bond which is stronger than the bond between the coating and the carrier web, and
6) peeling away the carrier web to leave the coating of graphics on the display surface.

In step 1) the liquid mixture can be applied by any conventional coating technique, e.g., screen printing, spray painting, or knife coating. By printing the liquid mixture onto the carrier web, the graphics can have exceedingly fine detail and may be applied in half tones and multiple colors. As do conventional printable inks of the prior art, the liquid mixture may include pigments, dyes, fillers, and/or other light-altering agents and may also contain ultraviolet light absorbers, antioxidants, flow-control agents and surfactants, some of which may also be light-altering agents. Particulate light-altering agents are preferred, being more resistant than are dyes to the transfer fluids used in step 3). Also, the light-altering characteristics of particulates are less likely to change over periods of time than are dyes. Light-altering particulates may be used in proportions up to the critical pigment volume concentration, but any lesser proportion is viable unless opacity is required.

The liquid mixture may comprise solids dissolved or dispersed in a volatile vehicle, whereupon step 2) involves evaporating the vehicle. Instead the liquid mixture may comprise polymerizable liquid monomers which in step 2) are polymerized in situ to a solid state. Such polymerization can be effected by heating or by exposure to actinic radiation and normally requires a suitable catalyst to be included in the liquid mixture.

Preferred as the flexible, low-adhesion carrier web are polyethylene, polypropylene, polyallomer, and polytetrafluoroethylene films which are known to have low affinity for resin coatings while being highly resistant to fluids which attack the binder resin. Each of these films is transparent, which makes it easier to position the graphics on a display surface. Polyethylene is preferred because of its low cost. Other useful plastic films tend to be more expensive than polyethylene and may have low-adhesion coatings which add to their expense. The plastic films may incorporate reinforcing fibers or fabrics. Plastic-coated paper is also useful.

The binder resin is a film-forming resin which preferably adheres well to most surfaces but is at least partially dissolved by an economical, readily available transfer fluid such as turpentine or mineral spirits. Useful binder resins include acrylics such as butyl methacrylate, vinyl acetate copolymers, polyamides, pulyurethanes, and other resins typically used in paints and coatings to promote adhesion. Preferably the binder resin has a Tukon hardness of less than 10.

The matrix resin is a film-forming resin which provides a polymeric network that is resistant to transfer fluids which at least partially dissolve the binder resin. The matrix and binder resins should be thoroughly mixed so that the matrix resin will prevent any smearing of the coating of graphics even if the transfer fluid should completely dissolve the binder resin. Preferred matrix resins are polyurethanes, cellulose containing polymers, and vinyl chloride copolymers. Both the matrix resin and the binder resin can be polyurethanes due to their wide range of solubilities. Polyurethanes made from mono-functional or low-molecular-weight reactants tend to have better solubility and hence to be useful as binder resins.

The transfer fluid applied in step 3) may completely dissolve the binder resin or it may merely soften and tackify the binder resin sufficiently to allow a bond to develop when in step 4) the wet graphics are pressed against a display surface. Preferred transfer fluids are characterized by high (above 8.5) or low (below 4.0) hydrogen bonding indices, because they tend not to attack preferred matrix resins. If a transfer fluid does attack a certain matrix resin, that problem can usually be averted by substituting a transfer fluid which may have the same hydrogen bonding index but a different solubility parameter. For example, toluene and turpentine have the same hydrogen bonding index (3.8), but toluene (solubility parameter of 8.9) attacks more resins than does turpentine (solubility parameter of 8.1). The hydrogen bonding index of mineral spirits is 2.2. Other useful transfer fluids include isopropyl alcohol and ethyl alcohol, each of which has a hydrogen bonding index of 8.9. Their solubility parameters are 11.5 and 13.6, respectively. Also shown to be useful is "Penola" 150 which is a mixture of aromatic hydrocarbons having a 65° C flashpoint, a hydrogen bonding index of about 3.8, and a solubility parameter of about 8.5.

The matrix resin may comprise as little as 2 % and as such as 50 % by weight of total matrix and binder resins, preferably at least 5 % when using a transfer fluid that dissolves binder resin. When the proportion of matrix resin is small, the amount of transfer-fluid preferably is limited to an amount barely sufficient to wet the entire coating of graphics. Usually the proportion of matrix resin is kept to the minimum that will assure no smearing of the coating of graphics, because high proportions of binder resin insure good adhesion to display surfaces. For this reason, the proportion of matrix resin preferably does not exceed 30 % by weight of total matrix and binder resins.

The solidified coating of graphics preferably has a thickness within the range of 0.0025 to 0.025 mm. Within that range, the graphics after being transferred to a display surface can have the appearance of exactingly applied paint, giving an aura of high quality. Below 0.0025 mm the graphics may involve transfer problems. Above 0.05 mm would usually be wasteful of raw materials.

Upon solidifying the coating in step 2), the carrier web and its coating of graphics provide a graphic transfer medium which can be wound upon itself for storage and shipment and can be used by retail merchants for applying the graphics to display surfaces such as windows. High quality graphics are obtainable, because they can be created at a central location for large numbers of merchants who need only to activate the binder resin with a transfer fluid in order to transfer the graphics to a display surface.

As indicated above, the graphics transfer medium of the invention may be most useful in enabling retail merchants to post visual announcements of high quality at low expense. However, the novel medium should have a number of other important uses. For example, it can be used to apply decorative and functional graphics to vehicular surfaces, and for such use the light-altering agent may comprise retroreflective beads. The novel medium also can be used wherever there is a need for graphics that are not noticably raised above a display surface.

### Brief Description of the Drawings

The invention is further explained with reference to the drawings wherein:
Figsre 1 is a shematic cross section of a graphics transfer medium of the invention; and
Figure 2 schematicaliy shows the use of the medium of Figure 1 to tranafer a coating of graphics to a display surface.

### Detailed Description

A graphics transfer medium 10 shown in Figure 1 includes a flexible low-adhesion carrier web 12 and a coating 14 of graphics. After wetting the coating 14 with a transfer fluid, the medium 10 has been applied to a display surface 20, as shown in Figure 2, and the carrier 12 is being peeled away to transfer the coating 14 of graphics to the display surface.

In the following examples, all parts and percentages are by weight unless otherwise stated.

### Example 1

The solids were added to the solvent according to recommendations of the raw material suppliers to yield a screen-printable ink having a viscosity of approximately 2500 mPa.s (2500 cps). This was screen-printed onto a transparent medium-density polyethylene carrier web approximately 0.125 mm thick. The screen printing was a test pattern including the alphabet, various geometric patterns, fine lines. and half tones. The coating was solidified by drying overnight in air to yield a dried thickness of approximately 0.01 mm.

The resulting graphic transfer medium could be wound upon itself into roll form for storage and shipment,

Turpentine transfer fluid was sprayed onto an aluminum panel in an amount barely sufficient to wet its surface. The coating of the medium was placed in contact with the wet surface and firmly rubbed down. After approximately 30 seconds, the polyethylene carrier web was stripped off leaving graphics which appeared to have the same quality as the original test pattern. After drying overnight, the graphics were resistant to scratching, moisture, and sunlight.

Other specimens of Example 1 were successfully transferred to polyester film, glass plate, polycarbonate shooting, polymethylmethacrylate sheet, and baked enamel metal panel.

### Examples 2-8

Graphics transfer media similar to that of Example 1 were prepared using transparent low-density polyethylene film as the flexible, low-adhesion carrier web. The ingredients of the coatings of graphics are indicated in parts by weight in Tables A and B except that Examples 5-8 included 0.015 part of the siloxane, 0.37 part of the fluorochemical, and 1.485 part of the xylene used in Example 1.

Used to transfer the graphics of Examples 2-8 to various substrates were

Additional graphics transfer media have been prepared which were identical to those of Examples 1-8 except by changing the percent of the matrix resin to total matrix and binder resins. Good results were demonstrated within the following ranges:

The graphics transferred from the medium of Example 4 could be peeled off various display surfaces such as glass plate, polyester film, and lacquered metal. The graphics transferred to such surfaces from the media of Examples 1-3 and 5-8 could not be removed intact.

When the light-altering agent was nearly colorless silica as in Example 8 and the graphics were transferred to a glass plate, the image looked very much like glass which had been etched.

## Claims

1.Method of applying graphics to a display surface comprising the sequential steps of
1) applying to a flexible, low-adhesion carrier web a coating in the form of graphics, which coating comprises a liquid mixture of
a) matrix resin,
b) binder resin, and
c) light-altering agent,
2) solidifying the coating of graphics,
3) wetting the solidified coating of graphics with fluid which at least partially dissolves the binder resin and substantially does not attack either the matrix resin or the carrier web,
4) pressing the wet coating of graphics against a display surface,
5) allowing to develop between the coating of graphics and the display surface a bond which is stronger than the bond between the coating and the carrier web, and
6) peeling away the carrier web to leave the coating of graphics on the display surface.

2. Method as defined in claim 1 wherein step 1) involves printing the liquid mixture onto the carrier web.

3. Method as defined in claim 2 wherein step 1) involves screen printing.

4. Method as defined in claim 1 wherein Step 1) involves spray painting said liquid mixture through a stencil onto the carrier web.

5. Method as defined in claim 1 wherein step 1) involved knife coating.

6. Method as defined in claim 1 wherein between steps 2) and 3) the coated carrier web is wound upon itself in roll form for storage or shipment.

7. Method as defined in claim 1 whehein the liquid mixture comprises volatile vehicle, and step 2) involves evaporating the vehicle.

8. Method as defined in claim 1 wherein step 3) involves applying the transfer fluid in an amount barely sufficient to wet the coating of graphics.

9. Method as defined in claim 1 wherein the matrix resin comprises from 2 to 50 percent by weight of total matrix and binder resins.

10. Method as defined in claim 9 wherein the matrix resin comprises from 5 to 30 percent by weight of total matrix and binder resins.

11. Method as defined in claim 1 wherein the light-altering agent comprises pigment.

12. A graphics transfer medium comprising a flexible low-adhesion carrier web carrying a coating in the form of graphics, which coating comprises a mixture of
a) matrix resin,
b) binder resin, and
c) light-altering agent,
which binder resin, when wet with a transfer fluid to which the matrix resin is resistant, is capable of forming a bond to a display surface sufficient to enable the coating of graphics to be transferred from the carrier web to the display surface..

13. A medium as defined in claim 12 wound upon itself in roll form for storage or shipment.

14. A medium as defined in claim 12 wherein the matrix resin comprises from 2 to 50 percent by weight of total matrix and binder resins.

15. A medium as defined in claim 14 wherein the matrix resin comprises from 5 to 30 percent by weight of total matrix and binder resins.

16. A medium as defined in claim 15 wherein the binder resin has a Tukon hardness of less than 10.

17. A medium as defined in claim 16 wherein the carrier web is transparent.

18. A medium as defined in claim 12 wherein the light-altering agent comprises pigment.

## Patentansprüche

1. Verfahren zum Aufbringen von Graphiken auf eine Bilddarstellungsfläche mit folgenden aufeinanderfolgenden Schritten:
1) Auf eine flexible, schwach haftfähige Trägerbahn wird in Form einer Graphik ein Überzug afugetragen, der mindestens teilweise aus einem flüssigen Gemisch aus
a) einem Grundmassenharz,
b) einem Bindemittelharz und
c) einem lichtändernden Mittel besteht;
2) der Graphiküberzug wird verfestigt;
3) der verfestigte Graphiküberzug wird mit einem Fluid benetzt, in dem sich das Bindemittelharz mindestens teilweise auflöst und das das Grundmassenharz und die Trägerbahn im wesentlichen nicht angreift;
4) der nasse Graphiküberzug wird gegen eine Bilddarstellungsfläche gedrückt;
5) zwischen dem Graphiküberzug und der Bilddarstellungsfläche wird die Entwicklung einer Bindung gestattet, die fester ist als die Bindung zwischen dem Überzug und der Trägerbahn, und
6) die Trägerbahn wird abgezogen, so daß der Graphiküberzug auf der Bilddarstellungsfläche zurückbleibt.

2. Verfahren nach Anspruch 1, dadurch gekennzeichnet, daß im Schritt 1) das flüssige Gemisch auf die Trägerbahn gedruckt wird.

3. Verfahren nach Anspruch 2, dadurch gekennzeichnet, daß im Schritt 1) einen Siebdruckvorgang umfaßt.

4. Verfahren nach Anspruch 1, dadurch gekennzeichnet, daß im Schritt 1) das genannte flüssige Gemisch durch eine Schablone auf die Trägerbahn gesprüht wird.

5. Verfahren nach Anspruch 1, dadurch gekennzeichnet, daß im Schritt 1) ein Auftragvorgang mit einer Rakel durchgeführt wird.

6. Verfahren nach Anspruch 1, dadurch gekennzeichnet, daß zwischen den Schritten 2) und 3) die überzogene Trägerbahn für die Lagerung oder den Versand auf sich selbst zu einer Rolle aufgewickelt wird.

7. Verfahren nach Anspruch 1, dadurch gekennzeichnet, daß das flüssige Gemisch ein flüchtiges Bindemittel enthält, das im Schritt 2) verdampft wird.

8. Verfahren nach Anspruch 1, dadurch gekennzeichnet, daß im Schritt 3) das Umdruckfluid nur in der zum Benetzen des Graphiküberzuges erforderlichen Menge aufgetragen wird.

9. Verfahren nach Anspruch 1, dadurch gekennzeichnet, daß die Menge des Grundmassenharzes 2 bis 50 Gew.% der Gesamtmenge des Grundmassen- und des Bindemittelharzes beträgt.

10. Verfahren nach Anspruch 9, dadurch gekennzeichnet, daß die Menge des Grundmassenharzes 5 bis 30 Gew.% der Gesamtmenge des Grundmassen- und des Bindemittelharzes beträgt.

11. Verfahren nach Anspruch 1, dadurch gekennzeichnet, daß das lichtändernde Mittel mindestens teilweise aus Pigment besteht.

12. Graphikumdruckmedium mit einer flexiblen, schwach haftfähigen Trägerhahn, die einen eine Graphik bildenden Überzug trägt, der mindestens teilweise aus einem Gemisch aus
a) Grundmassenharz,
b) Bindemittelharz und
c) einem lichtändernden Mittel
besteht, wobei das Bindemittelharz bei seiner Benetzung mit einem Umdruckfluid, gegenüber dem das Grundmassenharz beständig ist, geeignet ist, mit einer Bilddarstellungsfläche eine Bindung herzustellen, die genügt, um eine Übertragung des Graphiküberzuges von der Trägerbahn auf die Bilddarstellungsfläche zu gestatten.

13. Medium nach Anspruch 12, das für die Lagerung oder den Versand auf sich selbst zu einer Rolle aufgewickelt ist.

14. Medium nach Anspruch 12, dadurch gekennzeichnet, daß die Menge des Grundmassenharzes 2 bis 50 Gew.% der Gesamtmenge des Grundmassen- und des Bindemittelharzes beträgt.

15. Medium nach Anspruch 14, dadurch gekennzeichnet, daß die Menge des Grundmassenharzes 5 bis 30 Gew.% der Gesamtmenge des Grundmassen- und des Bindemittelharzes beträgt.

16. Medium nach Anspruch 15, dadurch gekennzeichnet, daß das Bindemittelharz eine Tukonhärte unter 10 besitzt.

17. Medium nach Anspruch 16, dadurch gekennzeichnet, daß die Trägerbahn durchsichtig ist.

18. Medium nach Anspruch 12, dadurch gekennzeichnet, daß das lichtändernde Mittel wenigstens teilweise aus Pigment besteht.

## Revendications

1. Procédé d'application de motifs graphiques à une surface d'affichage, comprenant les opérations séquentielles de:
1) application, à une feuille support flexible de faible adhérence, d'un revêtement sous la forme de motifs graphiques, ce revêtement comprenant un mélange liquide de:
a) résine de matrice,
b) résine de liant, et
c) agent de modification de la lumière
2) solidification du revêtement de motifs graphiques,
3) mouillage du revêtement solidifié de motifs graphiques avec un fluide qui dissout au moins partiellement le liant de résine et qui n'attaque pas sensiblement la résine de matrice ou la feuille support,
4) pressage du revêtement de motifs graphiques mouillé, contre une surface d'affichage,
5) développement d'une liaison, entre le revêtement de motifs graphiques et la surface d'affichage, qui est plus solide que la liaison entre le revêtement et la feuille support, et
6) décollement de la feuille support pour laisser le revêtement de motifs graphiques sur la surface d'affichage.

2. Procédé suivant la revendication 1, dans lequel l'opération 1) comprend l'impression du mélange liquide sur la feuille support.

3. Procédé suivant la revendication 2, dans lequel l'opération 1) comprend une impression à l'écran.

4. Procédé suivant la revendication 1, dans lequel l'opération 1) comprend la peinture par pulvérisation dudit mélange liquide au moyen d'un pochoir sur la feuille support.

5. Procédé suivant la revendication 1, dans lequel l'opération 1) comprend une application à la lame.

6. Procédé suivant la revendication 1, dans lequel, entre les opérations 2) et 3), la feuille support revêtue est enroulée sur elle-même sous forme de rouleau, pour le stockage ou le transport.

7. Procédé suivant la revendication 1, dans lequel le mélange liquide comprend un véhicule volatil, et l'opération 2) comprend l'évaporation du véhicule.

8. Procédé suivant la revendication 1, dans lequel l'opération 3) comporte l'application du fluide de transfert en une quantité juste suffisante pour mouiller le revêtement de motifs graphiques.

9. Procédé suivant la revendication 1, dans lequel la résine de matrice constitue de 2 à 50 % en poids de la totalité des résines de matrice et de liant.

10. Procédé suivant la revendication 9, dans lequel la résine de matrice constitue de 5 à 30 % en poids de la totalité des résines de matrice et de liant.

11. Procédé suivant la revendication 1, dans lequel l'agent de modification de la lumière est un pigment.

12. Support de transfert graphique comprenant une feuille support flexible de faible adhérence portant un revêtement sous la forme de motifs graphiques, ce revêtement étant un mélange de
a) résine de matrice,
b) résine de liant, et
c) agent de modification de la lumière,
ladite résine de liant, lorsqu'elle est mouillée avec un fluide de transfert auquel la résine de matrice résiste, pouvant former une liaison avec une surface d'affichage, suffisante pour permettre le transfert du revêtement de motifs graphiques de la feuille support à la surface d'affichage.

13. Support suivant la revendication 12, enroulé sur lui-même sous forme de rouleau pour le stockage ou le transport.

14. Support suivant la revendication 12, dans lequel la résine de matrice constitue de 2 à 50 % en poids de la totalité des résines de matrice et de liant.

15. Support suivant la revendication 14, dans lequel la résine de matrice constitue de 5 à 30 % en poids de la totalité des résines de matrice et de liant.

16. Support suivant la revendication 15, dans lequel la résine de liant a une dureté Tukon inférieure à 10.

17. Support suivant la revendication 16, dans lequel la feuille support est transparente.

18. Support suivant la revendication 12, dans lequel l'agent de modification de la lumière comprend un pigment.
